

## UNITED STATES PATENT OFFICE.

CHARLES JOSEPH MICHEL MARIE LE PETIT, OF PARIS, FRANCE, ASSIGNOR OF ONE-FIFTH TO JAMES STUART BURNS, OF LONDON, ENGLAND.

## TREATMENT OF HIDES, SKINS, AND THE LIKE.

No Drawing.

Application filed December 11, 1923. Serial No. 680,041.

The present invention is for improvements in and relating to the treatment of hides, skins, and the like, hereinafter referred to as hides, and has particular reference to the provision of a preliminary dressing process preparatory to tanning. The invention concerns that class of process in which the hide is treated in a bath containing the type of ferment known as enzymes.

10 The invention is based upon the discovery that if hides, skins or the like be treated with an enzyme bath as hereinafter set forth, there is produced, instead of a depleting action such as is so characteristic of 15 the use of tryptic and other animal ferments of like action, quite the reverse effect when the treated material is subsequently subjected to tanning. The leather is markedly thickened as well as being of 20 high quality and texture, and the purpose of that feature of the present invention which consists in a process of treatment of the hide or skin preparatory to and in conjunction with tanning is to facilitate the tanning 25 process and to obtain a finished product of the improved properties evidenced by increased thickness and weight and quality of leather, together with good tensile strength and wear, the combination of the preparatory and tanning processes swelling the 30 hide producing added weight, thickness and durability. The invention is particularly applicable to the treatment of heavy hides, and it will be appreciated that the extent 35 of improvement in respect of one or more of the properties mentioned is dependent upon the nature of the raw material, other conditions remaining the same.

According to this invention, the aforesaid 40 tanning preparatory process for the purpose described consists in treating the hide, skin or the like in an exclusively vegetable-derived lipolytic bath of acid reaction (preferably acid with an organic acid, such as 45 butyric or lactic acid) in presence of an agent or agents promotive of the lipolytic action of the ferments, such as a lipase activator (for example, a manganese salt, such as manganese sulphate), or a fat-emulsifying agent, (for example, an alkali sulphuricinate, such as sodium sulphuricinate).

Thus, the hide may be treated with the

liquor obtained by the fermentation in presence of a lipase activator of a vegetable 55 lipase-yielding material in an aqueous medium.

For example, the hide may be treated with a liquor (appropriately acidified as may be required, preferably with an organic acid 60 such as butyric- or lactic-acid) derived from the fermentation in presence of an activator such as manganese sulphate of castor-oil seeds or castor oil seed residues in water.

It is preferred to use castor-oil seeds as 65 pure and fresh as are obtainable. The seeds may be oil-extracted, and both the pulp and the shells may be used for preparing the bath, the use of the whole seed being preferred.

70 It has been found that an exclusively vegetable lipolytic enzyme bath possesses the property of facilitating the tanning operation and improving the quality of the leather produced thereby, but it does not 75 necessarily follow that the action of the bath in this respect is to be attributed solely to the lipolytic ferment, and other substances present in the material from which the lipolytic ferment is derived may play their part 80 in the process. The expression "vegetable-derived lipolytic bath" as used herein is therefore to be understood to include such a bath containing substances or enzymes derived from the ferment-yielding material in 85 addition to those whose specific action is to effect the hydrolysis of fats.

Prior to treatment in the preparatory bath, the hides should be cleaned from excess fat, and fleshy matters and from lime or 90 other depilatory agent which may have been used for dehauling. One method of doing this is by suspension of the hide for about six hours in a aqueous bath having about three-quarters of a pound of bisulphite of 95 sodium and one-quarter of a pound of butyric-acid per hundred pounds of water, the temperature of the bath being not less than 12° C. The process may be considerably expedited by effecting the treatment in a 100 drum. The hide for treatment in the tanning preparatory bath should be of neutral reaction or slightly acid, an organic acid being preferably employed as aforesaid.

105 The tanning preparatory process may be carried out at any desired temperature ac-

cording to circumstances, such as the nature of the hide under treatment. For some goods, the temperature of the bath may be from about 21 to 38° C., while in other cases, 5 e. g. generally for light weight goods, the most advantageous results, from the point of view of rapidity combined with a high quality product, may be generally obtained when the liquor is maintained at approximately 10 the same temperature as that of the "live" hide, that is, about 35 to 38° C.

The bath may advantageously contain a reagent, such as sodium fluoride, which possesses the property of inhibiting counter fermentations or putrefactive changes, and it will be frequently found advantageous to make a fresh addition of such reagent to the liquor prior to treatment therewith of a fresh batch of hides. When the latter are 15 in good condition, a comparatively small proportion of such a reagent, for example, one pound of sodium fluoride per ton of the liquor, will generally be found to be sufficient in order to maintain a normal fermentation. In the contrary case, or where at any stage in the process indications are shown of the commencement of putrefactive change, the proportion should be increased, for example, to eight-and-a-half pounds of 20 sodium fluoride per ton of the liquor, and increase in the quantity of such an inhibitive reagent is in any case a good precautionary measure as a general rule in hot weather.

35 Over-exposure to the action of the bath may result in shrinkage or like undesired change of the material, to the defeat of the aforementioned purpose of the preparatory treatment, and the latter is therefore to be 40 understood as conducted according to this invention only to such a stage as to achieve this purpose in contradistinction to depletion of the material. The goods should, consequently, be kept under careful observation, 45 being removed from time to time, as may be found necessary, for inspection. For some hides, with a well-fermented bath, one-half hour may suffice, while in the case of others one and one-half hours or more may 50 be required to give the desired aforementioned results, but as will be appreciated a rule applicable to all cases cannot be laid down, and the time may be varied according to the nature of the particular hide, and the 55 changes observed during treatment in the bath.

It is of course known in fermentation reactions to add a reagent inimical to putrefactive change to the reaction mixture, and 60 no claim is made herein to the general use of preservatives for this purpose.

The preferred preparatory bath is prepared by the fermentation of castor-oil seeds appropriately disintegrated, in an aqueous medium, with or without castor-oil, in pres-

ence of a lipase-activator, such, for example, as a manganese salt.

A fat-emulsifying agent may be added to the mixture (for example, an alkali sulphuricinate, such as sodium sulphuricinate) 70 or said agent may be added to the bath before introduction therein of the hide or the like.

The fermentation may be effected at a temperature substantially between 26 to 75 28° C.

For reasonably expeditious preparation, the proportion of the liquid component of the fermentation mixture should not exceed about four times the weight of seed-pulp. 80

After conclusion of the fermentation which, at the temperature stated, may take from 48 to 60 hours, the addition may be made to the liquor of a reagent such as sodium fluoride for the purpose previously 85 mentioned.

The liquor so obtained, with or without dilution, as may be found convenient, may be directly applied as a tanning preparatory bath. It is, however, preferred to utilize a 90 liquor which has been sown with a culture of lactic yeast, this addition appearing generally to improve the bath and the course of the reactions going forward therein. The latter may itself advantageously be "activated" prior to introduction into the lipase-liquor.

The activation of the yeast may be effected by growing the yeast in an aqueous culture medium containing a pulp of castor-oil 100 seeds. Alternatively, the yeast may be grown in an aqueous culture medium containing initially a very small proportion of sulphuricinate of sodium, the proportion of which is gradually increased. A small 105 quantity of castor-oil seed pulp may also be added to the culture sulphuricinate solution used for cultivating the yeast. A satisfactory degree of development is obtained by leaving the yeast culture to stand at a temperature of about 28° C. over a period of 110 from two to three days. The temperature control of the fermentation should be carefully observed.

This yeast culture may be added to the 115 liquor obtained by the fermentation of the castor-oil seeds, or may be added to the initial mixture prior to fermentation of the seeds. The latter procedure is to be preferred as then a strong and active lactic fermentation takes place in the bath from the commencement, and although this fermentation has little or no influence on the lipaseidic reaction, it tends to prevent counter fermentations during the ripening of the 120 bath.

In any event, the addition to the prepared bath of sodium fluoride or other reagent of similar properties is to be recommended.

In preparing a bath in one way according 130

to this invention, a mixture was made up as follows:—

5 Water 200 lbs.; castor-oil seeds in pulp 55½ lbs.; sodium sulphoricinate 2½ lbs.; manganese sulphate ½ to 1 oz.

This mixture was maintained at a temperature of about 26 to 28° C. for a period of about two days. The mixture was then 10 centrifuged, the mud and seed residues being preserved for the preparation of a fresh mixture, and to the liquor was added fluoride of sodium in the proportion of one pound of the salt per ton of liquor.

The treatment of the hide may be effected 15 by working the hide in the liquor, for example with a drum or paddle tumbler, in the customary manner, as may be desired. Among the results of treatment in a medium of this type is the digestion of fatty matters 20 and also of some of the protein constituents in the goods, and an opening of the pores of the material as well as an acceleration of the subsequent tanning process and, in general, an improvement in the quality of the material 25 finally obtained. The treated hide possesses an improved absorptive power for tanning extracts, a high degree of absorption, with consequent increase in thickness and weight of the hide as already referred 30 to, being effected by a materially shortened treatment, with the production of a well-cured and good wearing leather.

Acidification of the bath which, as previously mentioned, is preferably effected 35 with an organic acid, should be such as to maintain a slight acid reaction throughout the process of treatment of the hides and the like, and the acidity may be maintained by addition of acid during the process as may 40 be required. Where developing lactic yeast, or the fermentation product thereof is employed in the bath, it may not be necessary to make any further addition of organic acid in order to maintain an acid reaction.

45 Prior to treatment in the tanning preparatory bath the hide may be subjected to any desired preliminary dressing as is customary in the art. The hide may be dehaired by a desired process. Preferably, however, 50 depilation is effected by aqueous sodium sulphide and caustic alkali, the goods being thereafter treated with a solution of bisulphite of sodium in water, and then submitted to the action of a bath consisting essentially of an aqueous solution of an organic acid, such as formic, butyric, or acetic acid, to which may be added fluoride, with or without sodium chloride.

In effecting the tanning of the material 60 which has been submitted to the foregoing preparatory treatment, it is preferred to subject the goods to tanning liquors of regularly increasing specific gravity, say from about 0.5 to 12° Baumé, while the temperature 65 from beginning to end of the tanning

operations, that is to say in the handlers and in the drums and bark-tanning pits, is maintained substantially at 36° C.

The increase in specific gravity of the liquors is preferably 0.5° at a time, and the 70 period of treatment of the goods in successive liquors may be from one, two, three, or four hours up to eight hours.

Prior to introduction into the tanning liquor, the prepared material should be 75 washed, advantageously in a dilute alkali bath, e. g. one containing about two-and-a-half pounds of caustic soda per ton of water, the material being subsequently washed free from alkali with water or dilute acid. Alternatively, or in conjunction with one or more of these washings, it is recommended, particularly when the hides are to be tanned with tanning extracts, to put into the tanning drums a mixture of soluble mineral oil 85 (sulphonated mineral oil), sulphoricinate of soda, and an essential oil, such as turpentine, in substantially the proportions of

|                        | Kilos. |
|------------------------|--------|
| Soluble mineral oil    | 80     |
| Sulphoricinate of soda | 10     |
| Turpentine oil         | 3      |

per ton of hides under treatment. This addition should preferably be made during the 95 first period (of nine hours) of drumming and with a tannin extract of not more than 9° Baumé.

The tanning liquors may also contain a certain proportion of chloride of sodium, 100 and there may be added a liquid hydrocarbon, or chlorine derivative thereof, for example, petrol, carbon tetrachloride, acetylene tetrachloride, or bisulphide of carbon.

It has been found that by conducting the 105 tanning process under these conditions, not only is the quality of the leather improved, but the process is accelerated and the cost of production reduced. For instance, no subsequent drumming is necessary, and products are obtainable in a few weeks which by the usual method of production demand several months or, in some cases, even years for their preparation.

I claim:

1. A tanning preparatory process for the purpose described which consists in submitting the hide to the action of exclusively vegetable-derived lipolytic ferments in an acid medium in presence of an agent promotive of the lipolytic action of the ferments. 120

2. A tanning preparatory process for the purpose described which consists in submitting the hide to the action of exclusively vegetable-derived lipolytic ferments in an acid medium in presence of sodium fluoride and of an agent promotive of the lipolytic action of the ferments. 125

3. A tanning preparatory process for the purpose described which consists in submit- 130

- ting the hide to the action of exclusively vegetable-derived lipolytic ferments in an acid medium in presence of a lipase activator.
- 5 4. A tanning preparatory process for the purpose described which consists in submitting the hide to the action of exclusively vegetable-derived lipolytic ferments in an acid medium in presence of a lipase activator and a fat-emulsifying agent.
- 10 5. A tanning preparatory process for the purpose described which consists in submitting the hide to the action of exclusively vegetable-derived lipolytic ferments in an acid medium in presence of a lipase activator and an alkali sulphoricinate.
- 15 6. A tanning preparatory process for the purpose described which consists in submitting the hide to the action of exclusively vegetable-derived lipolytic ferments in an acid medium in presence of an agent promotive of the lipolytic action of the ferments and in presence of the fermentation products of lactic yeast.
- 20 7. A tanning preparatory process for the purpose described which consists in treating the hide with a bath of acid reaction derived from the prior fermentation in presence of a lipase activator of a vegetable lipase-yielding material in an aqueous medium.
- 25 8. A tanning preparatory process for the purpose described which consists in treating the hide with a bath of acid reaction derived from the prior fermentation in presence of a lipase activator of a vegetable lipase-yielding material in an aqueous medium, and containing sodium fluoride.
- 30 9. A tanning preparatory process for the purpose described which consists in treating the hide with a bath of acid reaction derived from the prior fermentation in presence of a lipase activator of a vegetable lipase-yielding material in an aqueous medium, and containing a fat-emulsifying agent.
- 35 10. A tanning preparatory process for the purpose described which consists in treating the hide with a bath of acid reaction derived from the prior fermentation in presence of a lipase activator of castor oil seeds in an aqueous medium.
- 40 11. A tanning preparatory process for the purpose described which consists in treating the hide with a bath of acid reaction derived from the prior fermentation in presence of manganese sulphate of castor oil seeds in an aqueous medium.
- 45 12. A tanning preparatory process for the purpose described which consists in treating the hide with a bath of acid reaction derived from the prior fermentation in presence of a lipase activator of castor oil seeds in an aqueous medium, and containing a fat-emulsifying agent.
- 50 13. A tanning preparatory process for the purpose described which consists in treating the hide with a bath of acid reaction derived from the prior fermentation in presence of a lipase activator of castor oil seeds in an aqueous medium, and containing 70
- 55 14. A tanning preparatory process for the purpose described which consists in treating the hide with a bath of acid reaction derived from the fermentation in presence of manganese sulphate of castor oil seeds in an aqueous medium, and containing 75
- 60 15. A tanning preparatory process for the purpose described which consists in treating the hide in a bath of acid reaction with an organic acid, derived from the prior fermentation in presence of a lipase activator of castor oil seeds in an aqueous medium.
- 65 16. A tanning preparatory process for the purpose described which consists in submitting the hide to the action of exclusively vegetable-derived lipolytic ferments in an acid medium in presence of an agent promotive of the lipolytic action of the ferments at a temperature corresponding substantially to that of the "live" hide.
- 70 17. A process of making a tanning preparatory liquor which consists in fermenting a vegetable lipase-yielding material in an aqueous medium in presence of a lipase activator.
- 75 18. A process of making a tanning preparatory liquor which consists in fermenting a mixture comprising water and disintegrated castor oil seed in presence of a lipase activator.
- 80 19. A process of making a tanning preparatory liquor which consists in fermenting a mixture comprising water and disintegrated castor oil seed in presence of manganese sulphate.
- 85 20. A process for making a tanning preparatory liquor which consists in fermenting in presence of a lipase activator and of a fat-emulsifying agent a vegetable-lipase-yielding material in an aqueous medium.
- 90 21. A process of making a tanning preparatory liquid which consists in fermenting a mixture comprising water, disintegrated castor oil seed, a lipase activator and an alkali sulphoricinate.
- 95 22. A process of making a tanning preparatory liquor which consists in fermenting in presence of a lipase activator a lipase-yielding material in an aqueous medium in the presence of developing lactic yeast.
- 100 23. A process of making a tanning preparatory liquor which consists in fermenting in presence of a lipase activator a mixture comprising water, disintegrated castor oil seed, and developing lactic yeast.
- 105 24. A process of making a tanning pre- 110
- 110 115
- 115 120
- 120 125
- 125 130

paratory liquor which consists in fermenting in presence of manganese sulphate a mixture comprising water and disintegrated castor oil seed at a temperature substantially between 26 and 28° C.

25. A process of making a tanning preparatory liquor which consists in fermenting in presence of manganese sulphate a mixture comprising water, disintegrated 10 castor oil seed, and developing lactic yeast at a temperature substantially between 26 and 28° C.

26. A process of making a tanning preparatory liquor which consists in fermenting 15 a mixture comprising water, disintegrated castor oil seed, an alkali sulphoricinate, and sulphate of manganese in substantially the proportions of 200 lbs. of water, 55½ lbs. of castor oil seed pulp, 2½ lbs. of the alkali 20 sulphoricinate, and one-fifth to 1 oz. of the manganese salt.

27. A process of making a tanning preparatory liquor which consists in growing lactic

yeast in a culture medium containing disintegrated castor oil seed, and then adding 25 the so-activated yeast culture to a mixture comprising water and disintegrated castor oil seed, and fermenting said mixture comprising the yeast culture in presence of manganese sulphate.

28. A process of making a tanning preparatory liquor which consists in growing lactic yeast in a culture medium initially containing a small proportion of an alkali sulphoricinate, and gradually increasing the 30 proportion of sulphoricinate during the growth of the yeast in the medium, and then adding the so-activated yeast culture to a mixture comprising water and disintegrated 35 castor oil seed and fermenting said mixture containing the yeast culture in presence of a manganese salt.

In testimony whereof I affix my signature.

CHARLES JOSEPH MICHEL MARIE LE PETIT.